

Sept. 23, 1952

T. R. THOMPSON  
PHOTOGRAPHIC EMULSIONS CONTAINING UNSYMMETRICAL  
TETRANUCLEAR CYANINE DYES

2,611,695

Original Filed Dec. 21, 1948

2 SHEETS—SHEET 1



Fig. 1.



Fig. 2.



Fig. 3.



INVENTOR  
Thomas R. Thompson

*Thomas R. Thompson*  
*Henry B. Fellows*  
ATTORNEYS

Sept. 23, 1952

T. R. THOMPSON  
PHOTOGRAPHIC EMULSIONS CONTAINING UNSYMMETRICAL  
TETRANUCLEAR CYANINE DYES

2,611,695

Original Filed Dec. 21, 1948

2 SHEETS—SHEET 2



Fig. 4.



Fig. 5.

INVENTOR  
Thomas R. Thompson  
BY *Henry B. Kellog*  
*Henry B. Kellog*  
ATTORNEYS

## UNITED STATES PATENT OFFICE

2,611,695

PHOTOGRAPHIC EMULSIONS CONTAINING  
UNSYMMETRICAL TETRANUCLEAR CY-  
ANINE DYESThomas R. Thompson, Binghamton, N. Y., as-  
signor to General Aniline & Film Corporation,  
New York, N. Y., a corporation of DelawareOriginal application December 21, 1948, Serial  
No. 66,575, now Patent No. 2,518,731, dated Au-  
gust 15, 1950. Divided and this application  
April 30, 1949, Serial No. 90,712

4 Claims. (Cl. 95—7)

1

This invention relates to photographic gelatino silver-halide emulsions, and more particularly to photographic emulsions sensitized by means of new unsymmetrical tetranuclear cyanine dyes containing two internal thiazole nuclei.

The use of sensitizing dyes, particularly in multilayer color film, poses many problems. It is known that sensitizing dyes operate by dyeing the silver-halide grain. To do this, they must be adsorbed to the silver-halide. If they are displaced from the silver-halide grains, they lose their effectiveness as sensitizers. It is also known that many color formers used in color photography have greater affinity for silver-halides than the sensitizers, and act to displace the same from the silver-halide grains. One must, therefore, select a sensitizer which will not be so displaced.

Another problem arises as regards the migration of the sensitizers from one emulsion to another. Where this ensues, color distortion is the inevitable result. Many proposals have been made dealing with the anchoring of compounds in silver-halide emulsions, the most noteworthy being the use of a long alkyl chain (see Wilmanns et al. United States Patent 2,186,849).

It is, therefore, necessary when providing sensitizers, particularly for color photography, to make certain that they have (1) the proper sensitizing power, (2) the ability to withstand displacement from silver-halide grains by color formers, and (3) the ability to resist diffusion from one sensitized emulsion to another.

Efforts which satisfy the last prerequisite, unfortunately, often lead to compounds which will not meet the first two tests. Thus, it is known that the sensitizing power of cyanine dyes varies with the substituent on the cyanine N-atoms. Where this substituent is alkyl, the power decreases as the chain length increases. Hence, if a long alkyl chain be used to anchor the dye in the emulsion, we end up with a product of little or no sensitizing power. The use of other expedients to anchor the dye, on the other hand, often gives products incapable of withstanding the displacement action of color formers insofar as the silver-halide grains are concerned. It is thus manifest that the provision of sensitizers having the necessary prerequisite is a difficult problem, to say the least.

It is known that many cyanine dyes sensitize photographic silver-halide emulsions to high red sensitivity. Most of these dyes, however, are not suitable for sensitizing silver-halide emulsions containing color coupling components. This is

2

thought to be due to a physical displacement which the sensitizing dye undergoes when color coupling components are added. That is, the sensitizer is adsorbed to the surface of the silver-halide grain, and then, with addition of color coupling component, is displaced therefrom. Moreover, most of the cyanine dyes are incompatible with silver-halide emulsion stabilizers, such as, for example, mercapto-substituted tetrazoles.

An object of the present invention is to provide photographic silver-halide emulsions with unsymmetrical tetranuclear sensitizing dyestuffs containing two internal thiazole nuclei.

15 A further object is to provide such dyes which are free from the disadvantages noted above.

Other objects and advantages of this invention will become apparent by reference to the following specification in which its preferred details and embodiments are described.

This invention is based on the discovery that unsymmetrical tetranuclear cyanine dyes containing two internal thiazole nuclei not only sensitize a photographic silver-halide emulsion to high red sensitivity, but are also compatible with color coupling components for the cyan dye image and with practically all emulsion stabilizers including the mercapto-substituted tetrazoles. In the latter combination, the sensitizing action of the dyes is not impaired nor diminished. In addition to these desirable characteristics, it has been further found that when the dyes are used in conjunction with color coupling components for the blue-green image, the spectral curves of 30 these dyes show a desirable gap in the green region of the spectrum, i. e., the dye sensitivity is more selective to the red spectral region. The sensitizing capacity of these dyes is not only maintained in the presence of color coupling components for the blue-green image, especially those components containing long alkyl chains, but is in part rendered more selective.

Some of the unsymmetrical tetranuclear cyanine dyes of this invention which sensitize emulsions to the regions of longer wavelengths, are of extreme value in the manufacture of infrared silver-halide emulsions which can be exposed through light yellow filters instead of the ordinarily used heavy gray filters in view of their low sensitizing power for the green, yellow and red. An additional advantage of these dyes is their ability to remain fixed in the layer in which they are originally deposited.

The unsymmetrical tetranuclear cyanine dyes fulfilling the above advantage are obtained in

excellent yield and in readily purifiable form by heating a thiazolone cyanine dye salt containing a reactive methylene group adjacent to a keto group with a thiazolone cyanine dye salt intermediate in a suitable solvent, such as an aliphatic alcohol, e. g., methyl, ethyl, n-propyl, isopropyl and the like, in the presence of a basic condensing agent such as trimethylamine, triethylamine, pyridine, methyl pyridine, ethyl pyridine, quinoline, potassium carbonate and the like, on a steam bath or by heating the reaction mixture at reflux for a period of 5 to 20 minutes.

The dyes obtained by the foregoing procedure are characterized by the following formula:



wherein R represents hydrogen or an alkyl group, e. g., methyl, ethyl, propyl, or butyl, R being only alkyl when n represents 1, R' and R'' which may be alike or different represent an alkyl, allyl, aryl, or aralkyl group, e. g., methyl, ethyl, propyl, phenyl, naphthyl, tolyl, benzyl, phenethyl, and the like, R''' and R<sup>IV</sup> which may be alike or different represent an aliphatic, aryl, or aralkyl radical, e. g., methyl, ethyl, propyl, butyl, hydroxyethyl, ethoxyethyl, phenyl, tolyl, naphthyl, benzyl, phenethyl, menaphthyl, and the like, n represents a positive integer of from 1 to 3, X represents an acid radical, e. g., chloride, bromide, iodide, or alkyl sulfate, alkyl p-toluene-sulfonate or perchlorate, Z' and Z'' represent the atoms necessary to complete a heterocyclic nucleus of the type contained in cyanine dyes, e. g., oxazoles, thiazoles, selenazoles, and their polycyclic homologues, such as those of the benzene, naphthalene, i. e., naphthiazole and perinaphthiazole, acenaphthene, and anthracene series, pyridine, and its polycyclic homologues, such as quinoline and  $\alpha$ - and  $\beta$ -naphthaquinolines, perinaphthiazoles, indolenines, diazines, such as pyrimidines and quinazolines, diazoles (e. g., thio- $\beta$ - $\beta'$ -diazole), oxazolines pyrrolines, thiazolones and selenazolines (the polycyclic compounds of these series being substituted if desired in the carbocyclic rings with one or more conventional groups, such as alkyl or aryl as below, amino, hydroxy, alkoxy, i. e., methoxy, ethoxy, etc., and methylenedioxy groups, or by halogen atoms, i. e., chlorine, bromine, etc.), Z' and Z'' being the same or different depending upon whether R<sub>1</sub> and R<sub>2</sub> are the same or different. In other words, Z' and Z'' may be the same if R<sub>1</sub> and R<sub>2</sub> are different. However, if R<sub>1</sub> and R<sub>2</sub> are the same then Z' and Z'' must be different.

The thiazolone dye intermediates utilized as the coreactant with the thiazolone cyanine dye salts are characterized by the following general formulae:



and



wherein R<sub>2</sub>, R<sub>3</sub>, and Z have the same values as R'', R''' and Z' respectively, and X has the same values as above, R<sub>4</sub> represents an aryl group of the benzene and naphthalene series, such as phenyl, chlorophenyl, diphenyl, tolyl, or naphthyl, R<sub>5</sub> represents either hydrogen or an acetyl

group, R<sub>6</sub> represents an alkyl or aralkyl group, e. g., methyl, ethyl, propyl, isopropyl, benzyl,  $\beta$ -phenethyl, and the like, R<sub>7</sub> represents an alkyl group, e. g., methyl, ethyl, propyl, isopropyl, butyl, isobutyl, etc. and n represents a positive integer of from 1 to 3, and Y represents the atoms necessary to complete a saturated heterocyclic nitrogenous nucleus, such as, for example, piperidine,  $\beta$ - or  $\gamma$ -pipecoline, pyrrolidine, morpholine, tetrahydroquinoline, and the like.

30 The dyestuff intermediates illustrated by Formulae *a* and *c* are prepared according to the method described in my copending application Serial No. 66,571, filed December 21, 1948, now United States Patent 2,535,992, and the intermediates illustrated by the second Formula *b* are prepared according to the method described in my copending application Serial No. 66,572, filed December 21, 1948, now United States Patent 2,536,987.

40 The dyestuff intermediates illustrated by Formula *a* are, in general, obtained by treating a diarylformamidine or its vinyllog, such as  $\beta$ -anilinoacrolein anil hydrochloride or glutaconic aldehyde dianil hydrochloride, in the presence of an acid condensing agent such as acetic anhydride, or in the presence of a basic condensing agent such as triethylamine, or piperidine, with a thiazolone cyanine dye.

45 The dyestuff intermediates illustrated by Formula *b* are obtained by treating a thiazolone cyanine dye with an aliphatic acid anhydride in the presence of a mixture of pyridine and triethylamine followed by treatment with phosphorus pentasulfide to yield the thio derivative which is subsequently alkylated with an alkylating agent in the usual way to yield the thioether derivative.

50 The thiazolone cyanine dyes utilized in preparing the foregoing intermediates and which are 60 condensed with the said intermediates are characterized by the following general formula:



wherein R<sub>2</sub>, R<sub>3</sub>, X and Z' have the same values as above, and are prepared according to the method 70 described in my copending application Serial No. 786,814, filed November 18, 1947, now United States Patent 2,536,986. In general, the method consists of condensing a substituted thioamide with an  $\alpha$ -halogen acetic acid. The compounds, 75 in view of their ketomethylene configuration,

undergo keto-enol tautomerism, i. e., the keto group enolizes to form a hydroxyl group.

The following examples describe the preparation of some of the thiazolone cyanine dye intermediates illustrated by Formulae *a* and *b* which are utilized in the preparation of the tetranuclear cyanine dyes.

*Example I*



A mixture of 5 grams of diphenylformamidine, 5 grams of the thiazolone cyanine dye of the following structure:



and 15 cc. of acetic anhydride was heated at 140° C. for 30 minutes. After cooling, the product was precipitated with ether and purified by dissolving it in a small amount of methanol followed by precipitation with ether. A yield of 5.9 grams of yellow-green crystals, having a melting point at 213-215° C. was obtained.

*Example II*



A mixture of 75 cc. of pyridine, 15 cc. of propionic anhydride, 15 cc. of triethylamine, and 15 grams of the thiazolone cyanine dye of the following structure:



was heated at 120° C. for 30 minutes. Fifteen grams of phosphorus pentasulfide were added in portions and the reaction mixture stirred at 120° C. for 30 minutes. The product was isolated by

pouring the reaction mixture into 300 cc. of 5% aqueous solution of potassium iodide. The product was purified by washing with water and subsequently grinding with acetone. A yield of 10.9 grams of yellow glistening crystals melting at 255-260° C. was obtained. The product was fused with 10 cc. of methyl sulfate at 95° C. for 10 minutes to yield a thick solution which upon treatment with an acetone solution of sodium iodide deposits yellow crystals.

*Example III*



A mixture of 75 cc. of pyridine, 10 cc. of propionic anhydride, 10 cc. of triethylamine, and 13 grams of the thiazolone cyanine dye of the following structure:



was heated with stirring at 120° C. for 20 minutes. During the course of 10 minutes, a total of 10 grams of phosphorus pentasulfide was added in portions at 120° C. After an additional 10 minutes of stirring at 120° C., the mixture was poured into cold water and stirred until the first formed oil solidified. The crude product was stirred with 300 cc. of a 10% aqueous solution of sodium hydroxide and purified by boiling out with isopropanol. There was obtained 10.2 grams of yellow powder which decomposes at about 200° C.

A mixture of 9.3 grams of the yellow powder and 10 grams of methyl p-toluenesulfonate was fused at 95° C. for 1 hour. After cooling, the product was washed with ether and dissolved in 10 cc. of warm acetone. The final product was precipitated as the iodide by adding 25 cc. of methanol containing 20% sodium iodide. The product was washed with water and purified by boiling out with isopropanol. A yield of 4.3 grams of a product melting at 225-228° C. was obtained.

*Example IV*



A mixture of 15 cc. of pyridine, 2 cc. of propionic anhydride, 2 cc. of triethylamine, and 2.0 grams

of the thiazolone cyanine dye of the following structure:



was heated at 120° C. for 3 minutes. There were then added 2 grams of phosphorus pentasulfide and the mixture heated at 115° C. for 15 minutes. A dark red oil was precipitated by the addition of 100 cc. of water and washed with water by decantation. The product was fused with 3 cc. of methyl sulfate at 95° C. for 10 minutes to yield 4.5 grams of a yellow-orange solution which may be employed in dye synthesis.

*Example V* (Continued from page 25)

**Example V** (Continued from page 25)



A mixture of 0.5 gram of the thiazolone cyanine dye of Example III, 0.3 gram of  $\beta$ -anilinoacrolein anil hydrochloride, 10 cc. of methanol, and 0.5 gram of piperidine was heated at reflux for 5 minutes. The reaction mixture was poured into 60 cc. of water containing 1 gram of potassium iodide. The crystals were separated and purified by boiling out with isopropyl alcohol. A yield of 0.4 gram of a product having a melting point of 270–271° C. was obtained. A methanol solution of the compound has an absorption maximum at 540  $\mu$ .

**Example VI**



A mixture of 2.85 grams of glutaconaldehyde dianil hydrochloride, 4.3 grams of the thiazolone cyanine dye of Example III, 1 cc. of piperidine and 50 cc. of methanol was heated at reflux for 30 minutes. The reaction mixture was poured into 300 cc. of water containing 5 grams of potassium iodide. The precipitated product was filtered and boiled out with isopropyl alcohol. A yield of 3.7 grams of a compound having a melting point of 195–198° C. was obtained. A methanol solution of the product has an absorption maximum at 624  $\mu$ .

*Example VII* (Continued from page 5)



A mixture of 25 grams of the thiazolone cyanine dye of Example I, 20 cc. of *n*-butyric anhydride, 100 cc. of pyridine, and 20 cc. of triethylamine was heated and stirred at 120° C. for 20 minutes. There were then added 20 grams phosphorus pentasulfide and stirring at 120° C. continued for 20 minutes. The reaction mixture was poured into 700 cc. of cold water. The resulting brown precipitate was filtered off, washed with water, and boiled out with 100 cc. of isopropyl alcohol. A yield of 20.9 grams of the dried and purified product was obtained. The compound



is presumed to be an inner salt characterized by the following formula:



A mixture of 2 grams of the above material and 2 grams of ethyl *p*-toluenesulfonate was fused at 95° C. for 30 minutes. The reaction mixture was dissolved in 30 cc. of hot acetone, and 10 cc. of a 10% solution of sodium iodide in acetone was added. After cooling, the crystals were separated and purified by boiling out with isopropyl alcohol. A yield of 1 gram of a product melting between 210–213° C. was obtained.

The anions of the foregoing thiazolone cyanine dye salt intermediates may be replaced by other anions, such as iodide, thiocyanate, or perchlorate.

rate, by treating an alcohol solution of the dye salt with an aqueous or aqueous-alcohol solution containing a sodium or potassium salt of the desired anions.

The following examples describe in detail the method of preparing the symmetrical and unsymmetrical tetranuclear cyanine dyes from the foregoing thiazolone cyanine dye salts and dye salt intermediates, but it is to be understood that they are given merely for the purpose of illustration. 5 10

tion and are not to be construed as limitative.

*Example VIII*



A mixture of 0.5 gram of the product of Example V, 20 cc. of methanol and 0.5 gram of tri-



A mixture of 0.3 gram of p-toluenesulfonate salt of the product of Example III, 0.3 gram of the thiazolone cyanine dye utilized in Example IV, 15 cc. of methanol, and 0.5 cc. of triethylamine was heated at reflux for 15 minutes. 20 cc. of 20% sodium bromide in methanol was added and the dye separated on cooling and was purified by boiling out with isopropyl alcohol. A yield of 0.4 gram of a product melting at 226-227° C. was obtained. A methanol solution of this dye absorbs with a maximum at 660 m $\mu$ . When incorporated into a bromoiodo photographic emulsion, the optical sensitization ranges from 580 to 760 m $\mu$  with a maximum at 725 m $\mu$ .

*Example IX.*



A mixture of 0.3 gram of the product of Example II, 0.3 gram of the thiazolone cyanine dye uti-



lized in Example III, 20 cc. of isopropyl alcohol, and 1 cc. of triethylamine was heated at reflux

for 10 minutes. Two cc. of 20% sodium iodide in methanol was added and the dye separated on cooling and was purified by boiling out with isopropyl alcohol. A yield of 0.5 gram of a product melting at 225-226° C. was obtained. In methanol solution this dye absorbs with a maximum at 627 m $\mu$ . The dye sensitizes a photographic emulsion with a maximum at 695 m $\mu$ .

*Example X*



A mixture of 0.5 gram of the product of Example V, 20 cc. of methanol and 0.5 gram of tri-



ethylamine, 0.4 gram of a thiazolone cyanine dye of the following structure:



were heated at reflux for 5 minutes. After cooling, the dye crystals were removed and purified by boiling out with isopropyl alcohol. A yield of 0.25 gram of a product melting at 237-239°C. was obtained. A methanol solution of the dye absorbs light with two maxima at 420 m $\mu$  and 734 m $\mu$ . The sensitization of a photographic emul-



sion is extended to 800 m $\mu$  with a maximum at 760 m $\mu$ .

*Example XI*



A mixture of 0.5 gram of the product of Example VI, 20 cc. of methanol, 0.5 cc. of triethyl-

## 11

amine, and 0.4 gram of a thiazolone dye having the following formula:



was heated at reflux for 5 minutes. After cooling, the reaction mixture was poured into an aqueous solution of potassium iodide, the dye was separated and purified by boiling out with isopropyl alcohol. A yield of 0.4 gram of a product melting at 214-218° C. was obtained. A methanol solution has absorption maxima at 447 and 811 m $\mu$ . When the dye is incorporated in a photographic emulsion the sensitization is extended to 900 m $\mu$  with a maximum at 850 m $\mu$ .

## Example XII



A mixture of 0.7 gram of the product of Example VII and 2 cc. of methyl sulfate was fused at 95° C. for 30 minutes. There were then added 25 cc. of isopropanol, 3 cc. of triethylamine and 0.4 gram of a thiazolone cyanine dye having the

40

following formula:



The resulting mixture was heated at reflux for 10 minutes. After cooling, the mixture was poured into an aqueous solution of sodium iodide, and the precipitated dye purified by boiling out with isopropanol. A yield of 0.3 gram of a dye melting at 244-251° C. was obtained. A methanol solution of the dye had an absorption maximum at 623 m $\mu$ . When added to a photographic silver-halide emulsion, the dye extends the range of sensitization to 735 m $\mu$  with a maximum at 700 m $\mu$ .

The diagrammatic spectrograms constituting the accompanying drawing illustrate the regions of the spectrum to which some of the tri-nuclear cyanine dyes will sensitize a gelatino silver-halide emulsion containing about 4-5% of silver-halide and the extent of the sensitization at various wavelengths. Figures 1 to 5 of this drawing illustrate the sensitizing properties of

75

the dyes prepared in accordance with Examples VIII, IX, X, XI, and XIII, respectively.

This application is a division of my copending application Serial No. 66,575, filed December 21, 1948, now United States Patent 2,518,731.

It is evident from the foregoing examples that the procedure employed in the preparation of tetranuclear cyanine dyes is simple and requires a shorter period of time. By merely choosing from a wide variety of thiazolone cyanine dye and dye intermediates, both symmetrical and unsymmetrical tetranuclear cyanine dyes are obtained in excellent yield and in readily purifiable form.

15 While I have disclosed the preferred embodiments of my invention and the preferred modes of carrying the same into effect, it will be readily apparent to those skilled in the art that many variations may be made therein without departing from the spirit thereof. Accordingly, the scope of my invention is to be limited solely by the appended claims.

21

I claim:

1. A photographic gelatino silver-halide emulsion containing an unsymmetrical tetranuclear cyanine dyestuff of the following general formula:



wherein  $n$  represents a positive integer of from 1 to 3, R is selected from the class consisting of 50 hydrogen and lower alkyl, R being only lower alkyl when  $n$  represents 1, R' and R'' are selected from the class consisting of lower alkyl, allyl, aryl and aralkyl groups of the benzene and naphthalene series R''' and R<sup>IV</sup> are selected from the class consisting of lower alkyl, lower hydroxy-alkyl, lower alkoxyalkyl, aryl and aralkyl groups of the benzene and naphthalene series, X represents an acid radical, Z' and Z'' represent the atoms necessary to complete a heterocyclic nitrogenous system, and wherein at least one of the groups of radicals R'-R'' and Z'-Z'' are dissimilar.

70 2. A photographic gelatino silver-halide emul-

sion containing an unsymmetrical tetranuclear cyanine dyestuff of the following structure:



3. A photographic gelatino silver-halide emulsion containing an unsymmetrical tetranuclear cyanine dyestuff of the following structure:



4. A photographic gelatino silver-halide emulsion containing an unsymmetrical tetranuclear cyanine dyestuff of the following structure:



THOMAS R. THOMPSON.

#### REFERENCES CITED

The following references are of record in the file of this patent:

#### UNITED STATES PATENTS

| Number    | Name           | Date          |
|-----------|----------------|---------------|
| 2,263,018 | Sprague        | Nov. 18, 1941 |
| 2,395,879 | Kendall et al. | Mar. 5, 1946  |